



US009404203B2

(12) **United States Patent**  
**Gilmore et al.**

(10) **Patent No.:** **US 9,404,203 B2**  
(45) **Date of Patent:** **Aug. 2, 2016**

(54) **WRAPPED YARNS FOR USE IN ROPES HAVING PREDETERMINED SURFACE CHARACTERISTICS**

(71) Applicant: **Samson Rope Technologies**, Ferndale, WA (US)

(72) Inventors: **Justin Gilmore**, Lafayette, LA (US); **David E. O'Neal**, Lafayette, LA (US); **Danielle D. Stenvers**, Ferndale, WA (US); **Chia-te Chou**, Bellingham, WA (US); **Ronald L. Bryant**, Lafayette, LA (US); **Eric W. McCorkle**, Bellingham, WA (US)

(73) Assignee: **Samson Rope Technologies**, Ferndale, WA (US)

(\*) Notice: Subject to any disclaimer, the term of this patent is extended or adjusted under 35 U.S.C. 154(b) by 137 days.

(21) Appl. No.: **14/262,600**

(22) Filed: **Apr. 25, 2014**

(65) **Prior Publication Data**

US 2014/0230635 A1 Aug. 21, 2014

**Related U.S. Application Data**

(63) Continuation of application No. 13/466,994, filed on May 8, 2012, now Pat. No. 8,707,668, which is a continuation of application No. 12/815,363, filed on Jun. 14, 2010, now Pat. No. 8,171,713, which is a

(Continued)

(51) **Int. Cl.**

**D02G 3/38** (2006.01)  
**D02G 3/04** (2006.01)

(Continued)

(52) **U.S. Cl.**

CPC ..... **D02G 3/38** (2013.01); **D02G 3/047** (2013.01); **D02G 3/442** (2013.01); **D07B 1/02** (2013.01);

(Continued)

(58) **Field of Classification Search**

CPC ..... D02G 3/38; D02G 3/442; D02G 3/047; D07B 5/06; D07B 5/005; D07B 1/02; D07B 1/025

See application file for complete search history.

(56) **References Cited**

**U.S. PATENT DOCUMENTS**

429,174 A 6/1890 Ogilvy  
568,531 A 9/1896 Harthan

(Continued)

**FOREIGN PATENT DOCUMENTS**

CA 2019499 2/2002  
DE 7315621 10/1973

(Continued)

**OTHER PUBLICATIONS**

Pultrusion Industry Council, <http://www.acmanet.org/pic/products/description.htm>, "products & process: process description", 2001, 2 pages.

(Continued)

*Primary Examiner* — Shaun R Hurley

(74) *Attorney, Agent, or Firm* — Michael R. Schacht; Schacht Law Office, Inc.

(57) **ABSTRACT**

A blended yarn comprises a plurality of first fibers and a plurality of second fibers. A coefficient of friction of the second fibers is greater than a coefficient of friction of the first fibers. Abrasion resistance characteristics of the second fibers are greater than abrasion resistance properties of the first fibers. A gripping ability of the second fibers is greater than a gripping ability of the first fibers. The plurality of second fibers are combined with the plurality of first fibers such that the first fibers extend along the length of the blended yarn and the second fibers do not extend along the length of the blended yarn at least a portion of the second fibers are engaged with and extend from the plurality of first fibers effectively to define surface characteristics of the blended yarn.

**19 Claims, 5 Drawing Sheets**



**Related U.S. Application Data**

|                                                                                                                                                                                                                                                                                                         |             |         |                         |
|---------------------------------------------------------------------------------------------------------------------------------------------------------------------------------------------------------------------------------------------------------------------------------------------------------|-------------|---------|-------------------------|
| continuation of application No. 12/151,467, filed on May 6, 2008, now Pat. No. 7,735,308, which is a continuation of application No. 11/599,817, filed on Nov. 14, 2006, now Pat. No. 7,367,176, which is a continuation of application No. 10/903,130, filed on Jul. 30, 2004, now Pat. No. 7,134,267. | 3,977,172 A | 8/1976  | Kerawalla               |
|                                                                                                                                                                                                                                                                                                         | 3,979,545 A | 9/1976  | Braus et al.            |
|                                                                                                                                                                                                                                                                                                         | 4,022,010 A | 5/1977  | Gladenbeck et al.       |
|                                                                                                                                                                                                                                                                                                         | 4,031,121 A | 6/1977  | Brown                   |
|                                                                                                                                                                                                                                                                                                         | 4,036,101 A | 7/1977  | Burnett                 |
|                                                                                                                                                                                                                                                                                                         | 4,050,230 A | 9/1977  | Senoo et al.            |
|                                                                                                                                                                                                                                                                                                         | 4,056,928 A | 11/1977 | de Vries                |
|                                                                                                                                                                                                                                                                                                         | 4,099,750 A | 7/1978  | McGrew                  |
|                                                                                                                                                                                                                                                                                                         | 4,116,481 A | 9/1978  | Raue                    |
|                                                                                                                                                                                                                                                                                                         | 4,155,394 A | 5/1979  | Shepherd et al.         |
|                                                                                                                                                                                                                                                                                                         | 4,159,618 A | 7/1979  | Sokaris                 |
|                                                                                                                                                                                                                                                                                                         | 4,170,921 A | 10/1979 | Repass                  |
|                                                                                                                                                                                                                                                                                                         | 4,173,113 A | 11/1979 | Snellman et al.         |
|                                                                                                                                                                                                                                                                                                         | 4,184,784 A | 1/1980  | Killian                 |
|                                                                                                                                                                                                                                                                                                         | 4,195,113 A | 3/1980  | Brook                   |
|                                                                                                                                                                                                                                                                                                         | 4,202,164 A | 5/1980  | Simpson et al.          |
|                                                                                                                                                                                                                                                                                                         | 4,210,089 A | 7/1980  | Lindahl                 |
|                                                                                                                                                                                                                                                                                                         | 4,226,035 A | 10/1980 | Saito                   |
|                                                                                                                                                                                                                                                                                                         | 4,228,641 A | 10/1980 | O'Neil                  |
|                                                                                                                                                                                                                                                                                                         | 4,232,619 A | 11/1980 | Lindahl                 |
|                                                                                                                                                                                                                                                                                                         | 4,232,903 A | 11/1980 | Welling et al.          |
|                                                                                                                                                                                                                                                                                                         | 4,250,702 A | 2/1981  | Gundlach                |
|                                                                                                                                                                                                                                                                                                         | 4,257,221 A | 3/1981  | Feinberg                |
|                                                                                                                                                                                                                                                                                                         | 4,258,608 A | 3/1981  | Brown                   |
|                                                                                                                                                                                                                                                                                                         | 4,286,429 A | 9/1981  | Lin                     |
|                                                                                                                                                                                                                                                                                                         | 4,312,260 A | 1/1982  | Morieras                |
|                                                                                                                                                                                                                                                                                                         | 4,321,854 A | 3/1982  | Foote et al.            |
|                                                                                                                                                                                                                                                                                                         | 4,329,794 A | 5/1982  | Rogers                  |
|                                                                                                                                                                                                                                                                                                         | 4,350,380 A | 9/1982  | Williams                |
|                                                                                                                                                                                                                                                                                                         | 4,375,779 A | 3/1983  | Fischer                 |
|                                                                                                                                                                                                                                                                                                         | 4,403,884 A | 9/1983  | Barnes                  |
|                                                                                                                                                                                                                                                                                                         | 4,412,474 A | 11/1983 | Hara                    |
|                                                                                                                                                                                                                                                                                                         | 4,421,352 A | 12/1983 | Raue et al.             |
|                                                                                                                                                                                                                                                                                                         | 4,464,812 A | 8/1984  | Crook, Jr. et al.       |
|                                                                                                                                                                                                                                                                                                         | 4,500,593 A | 2/1985  | Weber                   |
|                                                                                                                                                                                                                                                                                                         | 4,509,233 A | 4/1985  | Shaw                    |
|                                                                                                                                                                                                                                                                                                         | 4,534,163 A | 8/1985  | Schuerch                |
|                                                                                                                                                                                                                                                                                                         | 4,534,262 A | 8/1985  | Swenson                 |
|                                                                                                                                                                                                                                                                                                         | 4,563,869 A | 1/1986  | Stanton                 |
|                                                                                                                                                                                                                                                                                                         | 4,606,183 A | 8/1986  | Riggs                   |
|                                                                                                                                                                                                                                                                                                         | 4,619,108 A | 10/1986 | Hotta                   |
|                                                                                                                                                                                                                                                                                                         | 4,635,989 A | 1/1987  | Tremblay et al.         |
|                                                                                                                                                                                                                                                                                                         | 4,640,179 A | 2/1987  | Cameron                 |
|                                                                                                                                                                                                                                                                                                         | 4,642,854 A | 2/1987  | Kelly et al.            |
|                                                                                                                                                                                                                                                                                                         | 4,674,801 A | 6/1987  | DiPaola et al.          |
|                                                                                                                                                                                                                                                                                                         | 4,677,818 A | 7/1987  | Honda et al.            |
|                                                                                                                                                                                                                                                                                                         | 4,757,719 A | 7/1988  | Franke                  |
|                                                                                                                                                                                                                                                                                                         | 4,762,583 A | 8/1988  | Kaempen                 |
|                                                                                                                                                                                                                                                                                                         | 4,779,411 A | 10/1988 | Kendall                 |
|                                                                                                                                                                                                                                                                                                         | 4,784,918 A | 11/1988 | Klett et al.            |
|                                                                                                                                                                                                                                                                                                         | 4,850,629 A | 7/1989  | St. Germain             |
|                                                                                                                                                                                                                                                                                                         | 4,856,837 A | 8/1989  | Hammersla, Jr.          |
|                                                                                                                                                                                                                                                                                                         | 4,868,041 A | 9/1989  | Yamagishi et al.        |
|                                                                                                                                                                                                                                                                                                         | 4,887,422 A | 12/1989 | Klees et al.            |
|                                                                                                                                                                                                                                                                                                         | 4,947,917 A | 8/1990  | Noma et al.             |
|                                                                                                                                                                                                                                                                                                         | 4,958,485 A | 9/1990  | Montgomery et al.       |
|                                                                                                                                                                                                                                                                                                         | 4,974,488 A | 12/1990 | Spralja                 |
|                                                                                                                                                                                                                                                                                                         | 4,978,360 A | 12/1990 | Devanathan              |
|                                                                                                                                                                                                                                                                                                         | 5,060,466 A | 10/1991 | Matsuda et al.          |
|                                                                                                                                                                                                                                                                                                         | 5,091,243 A | 2/1992  | Tolbert et al.          |
|                                                                                                                                                                                                                                                                                                         | 5,141,542 A | 8/1992  | Fangeat et al.          |
|                                                                                                                                                                                                                                                                                                         | 5,178,923 A | 1/1993  | Andrieu et al.          |
|                                                                                                                                                                                                                                                                                                         | 5,211,500 A | 5/1993  | Takaki et al.           |
|                                                                                                                                                                                                                                                                                                         | D338,171 S  | 8/1993  | Bichi                   |
|                                                                                                                                                                                                                                                                                                         | 5,240,769 A | 8/1993  | Ueda et al.             |
|                                                                                                                                                                                                                                                                                                         | 5,288,552 A | 2/1994  | Hollenbaugh, Jr. et al. |
|                                                                                                                                                                                                                                                                                                         | 5,296,292 A | 3/1994  | Butters                 |
|                                                                                                                                                                                                                                                                                                         | 5,327,714 A | 7/1994  | Stevens et al.          |
|                                                                                                                                                                                                                                                                                                         | 5,333,442 A | 8/1994  | Berger                  |
|                                                                                                                                                                                                                                                                                                         | 5,378,522 A | 1/1995  | Lagomarsino             |
|                                                                                                                                                                                                                                                                                                         | 5,426,788 A | 6/1995  | Meltzer                 |
|                                                                                                                                                                                                                                                                                                         | 5,429,869 A | 7/1995  | McGregor et al.         |
|                                                                                                                                                                                                                                                                                                         | 5,441,790 A | 8/1995  | Ratigan                 |
|                                                                                                                                                                                                                                                                                                         | 5,483,911 A | 1/1996  | Kubli                   |
|                                                                                                                                                                                                                                                                                                         | 5,497,608 A | 3/1996  | Matsumoto et al.        |
|                                                                                                                                                                                                                                                                                                         | 5,501,879 A | 3/1996  | Murayama                |
|                                                                                                                                                                                                                                                                                                         | 5,506,043 A | 4/1996  | Lilani                  |
|                                                                                                                                                                                                                                                                                                         | 5,525,003 A | 6/1996  | Williams et al.         |
|                                                                                                                                                                                                                                                                                                         | 5,636,506 A | 6/1997  | Yngvesson               |

**(56) References Cited****U.S. PATENT DOCUMENTS**

|             |         |                        |
|-------------|---------|------------------------|
| 1,257,398 A | 2/1918  | Roach                  |
| 1,479,865 A | 1/1924  | Metcalf                |
| 1,490,387 A | 4/1924  | Hansen                 |
| 1,695,480 A | 12/1928 | Buoy                   |
| 1,710,740 A | 4/1929  | Ljungkull              |
| 1,769,945 A | 7/1930  | Erkert                 |
| 1,833,587 A | 11/1931 | Page                   |
| 1,850,767 A | 3/1932  | Page                   |
| 1,908,686 A | 5/1933  | Burke                  |
| 1,931,808 A | 10/1933 | Andersen               |
| 2,070,362 A | 2/1937  | Kreutz                 |
| 2,074,956 A | 3/1937  | Carstarphen            |
| 2,245,824 A | 6/1941  | Roesch                 |
| 2,299,568 A | 10/1942 | Dickey                 |
| 2,338,831 A | 1/1944  | Whitcomb et al.        |
| 2,359,424 A | 10/1944 | Joy                    |
| 2,480,005 A | 8/1949  | Ewell                  |
| 2,840,983 A | 7/1958  | Kelbach                |
| 2,960,365 A | 11/1960 | Meisen                 |
| 3,035,476 A | 5/1962  | Fogden                 |
| 3,073,209 A | 1/1963  | Benk et al.            |
| 3,276,810 A | 10/1966 | Antell                 |
| 3,358,434 A | 12/1967 | McCann                 |
| 3,367,095 A | 2/1968  | Field, Jr.             |
| 3,371,476 A | 3/1968  | Costello et al.        |
| 3,383,849 A | 5/1968  | Stirling               |
| 3,411,400 A | 11/1968 | Morieras et al.        |
| 3,415,052 A | 12/1968 | Stanton                |
| 3,425,737 A | 2/1969  | Sutton                 |
| RE26,704 E  | 11/1969 | Norton                 |
| 3,481,134 A | 12/1969 | Whewell, Jr.           |
| 3,507,949 A | 4/1970  | Campbell               |
| 3,537,742 A | 11/1970 | Black                  |
| 3,561,318 A | 2/1971  | Andriot, Jr.           |
| 3,653,295 A | 4/1972  | Pintard                |
| 3,662,533 A | 5/1972  | Snellman et al.        |
| 3,718,945 A | 3/1973  | Brindejonc de Treglode |
| 3,729,920 A | 5/1973  | Sayers et al.          |
| 3,762,865 A | 10/1973 | Weil                   |
| 3,771,305 A | 11/1973 | Barnett                |
| 3,839,207 A | 10/1974 | Weil                   |
| 3,854,767 A | 12/1974 | Burnett                |
| 3,904,458 A | 9/1975  | Wray                   |
| 3,906,136 A | 9/1975  | Weil                   |
| 3,915,618 A | 10/1975 | Feucht et al.          |
| 3,943,644 A | 3/1976  | Walz                   |
| 3,957,923 A | 5/1976  | Burke                  |
| 3,968,725 A | 7/1976  | Holzhauer              |

| (56)                                                                                                                                                             | References Cited |                   |                 |        |                       |
|------------------------------------------------------------------------------------------------------------------------------------------------------------------|------------------|-------------------|-----------------|--------|-----------------------|
| U.S. PATENT DOCUMENTS                                                                                                                                            |                  |                   |                 |        |                       |
| 5,643,516 A                                                                                                                                                      | 7/1997           | Raza et al.       | 2004/0069132 A1 | 4/2004 | Knudsen et al.        |
| 5,651,572 A                                                                                                                                                      | 7/1997           | St. Germain       | 2005/0036750 A1 | 2/2005 | Triplett et al.       |
| 5,669,214 A                                                                                                                                                      | 9/1997           | Kopanakis         | 2005/0172605 A1 | 8/2005 | Vancompernolle et al. |
| 5,699,657 A                                                                                                                                                      | 12/1997          | Paulson           | 2006/0048494 A1 | 3/2006 | Wetzel et al.         |
| 5,711,243 A                                                                                                                                                      | 1/1998           | Dunham            | 2006/0115656 A1 | 6/2006 | Martin                |
| 5,718,532 A                                                                                                                                                      | 2/1998           | Mower             | 2006/0179619 A1 | 8/2006 | Pearce et al.         |
| 5,727,833 A                                                                                                                                                      | 3/1998           | Coe               | 2006/0213175 A1 | 9/2006 | Smith et al.          |
| 5,802,839 A                                                                                                                                                      | 9/1998           | Van Hook          | 2007/0079695 A1 | 4/2007 | Bucher et al.         |
| 5,822,791 A                                                                                                                                                      | 10/1998          | Baris             |                 |        |                       |
| 5,826,421 A                                                                                                                                                      | 10/1998          | Wilcox et al.     |                 |        |                       |
| 5,852,926 A                                                                                                                                                      | 12/1998          | Breedlove         |                 |        |                       |
| 5,873,758 A                                                                                                                                                      | 2/1999           | Mullins           |                 |        |                       |
| 5,904,438 A                                                                                                                                                      | 5/1999           | Vaseghi et al.    |                 |        |                       |
| 5,931,076 A                                                                                                                                                      | 8/1999           | Ryan              |                 |        |                       |
| 5,943,963 A                                                                                                                                                      | 8/1999           | Beals             |                 |        |                       |
| 5,978,638 A                                                                                                                                                      | 11/1999          | Tanaka et al.     |                 |        |                       |
| 6,015,618 A                                                                                                                                                      | 1/2000           | Orima             |                 |        |                       |
| 6,033,213 A                                                                                                                                                      | 3/2000           | Halvorsen, Jr.    |                 |        |                       |
| 6,045,571 A                                                                                                                                                      | 4/2000           | Hill et al.       |                 |        |                       |
| 6,085,628 A                                                                                                                                                      | 7/2000           | Street et al.     |                 |        |                       |
| 6,122,847 A                                                                                                                                                      | 9/2000           | Treu et al.       |                 |        |                       |
| 6,146,759 A                                                                                                                                                      | 11/2000          | Land              |                 |        |                       |
| 6,164,053 A                                                                                                                                                      | 12/2000          | O'Donnell et al.  |                 |        |                       |
| 6,265,039 B1                                                                                                                                                     | 7/2001           | Drinkwater et al. |                 |        |                       |
| 6,295,799 B1                                                                                                                                                     | 10/2001          | Baranda           |                 |        |                       |
| 6,341,550 B1                                                                                                                                                     | 1/2002           | White             |                 |        |                       |
| 6,365,070 B1                                                                                                                                                     | 4/2002           | Stowell et al.    |                 |        |                       |
| 6,405,519 B1                                                                                                                                                     | 6/2002           | Shaikh et al.     |                 |        |                       |
| 6,410,140 B1                                                                                                                                                     | 6/2002           | Land et al.       |                 |        |                       |
| 6,422,118 B1                                                                                                                                                     | 7/2002           | Edwards           |                 |        |                       |
| 6,484,423 B1                                                                                                                                                     | 11/2002          | Murray            |                 |        |                       |
| 6,524,690 B1                                                                                                                                                     | 2/2003           | Dyksterhouse      |                 |        |                       |
| 6,575,072 B2                                                                                                                                                     | 6/2003           | Pellerin          |                 |        |                       |
| 6,592,987 B1                                                                                                                                                     | 7/2003           | Sakamoto          |                 |        |                       |
| 6,601,378 B1                                                                                                                                                     | 8/2003           | Fritsch et al.    |                 |        |                       |
| 6,704,535 B2                                                                                                                                                     | 3/2004           | Kobayashi et al.  |                 |        |                       |
| 6,876,798 B2                                                                                                                                                     | 4/2005           | Triplett et al.   |                 |        |                       |
| 6,881,793 B2                                                                                                                                                     | 4/2005           | Sheldon et al.    |                 |        |                       |
| 6,916,533 B2                                                                                                                                                     | 7/2005           | Simmelink et al.  |                 |        |                       |
| 6,945,153 B2                                                                                                                                                     | 9/2005           | Knudsen et al.    |                 |        |                       |
| 7,127,878 B1                                                                                                                                                     | 10/2006          | Wilke et al.      |                 |        |                       |
| 7,134,267 B1                                                                                                                                                     | 11/2006          | Gilmore et al.    |                 |        |                       |
| 7,137,617 B2                                                                                                                                                     | 11/2006          | Sjostedt          |                 |        |                       |
| 7,165,485 B2                                                                                                                                                     | 1/2007           | Smeets et al.     |                 |        |                       |
| 7,168,231 B1                                                                                                                                                     | 1/2007           | Chou et al.       |                 |        |                       |
| 7,172,878 B1                                                                                                                                                     | 2/2007           | Nowak et al.      |                 |        |                       |
| 7,182,900 B2                                                                                                                                                     | 2/2007           | Schwamborn et al. |                 |        |                       |
| 7,331,269 B2                                                                                                                                                     | 2/2008           | He et al.         |                 |        |                       |
| 7,367,176 B1                                                                                                                                                     | 5/2008           | Gilmore et al.    |                 |        |                       |
| 7,389,973 B1                                                                                                                                                     | 6/2008           | Chou et al.       |                 |        |                       |
| 7,437,869 B1                                                                                                                                                     | 10/2008          | Chou et al.       |                 |        |                       |
| 7,637,549 B2                                                                                                                                                     | 12/2009          | Hess              |                 |        |                       |
| 7,735,308 B1                                                                                                                                                     | 6/2010           | Gilmore et al.    |                 |        |                       |
| 7,743,596 B1                                                                                                                                                     | 6/2010           | Chou et al.       |                 |        |                       |
| 8,707,668 B2                                                                                                                                                     | 4/2014           | Gilmore et al.    |                 |        |                       |
| 8,717,713 B1                                                                                                                                                     | 5/2014           | Bjorstrom et al.  |                 |        |                       |
| 2003/0200740 A1                                                                                                                                                  | 10/2003          | Tao et al.        |                 |        |                       |
| 2003/0226347 A1                                                                                                                                                  | 12/2003          | Smith et al.      |                 |        |                       |
| 2004/0025486 A1                                                                                                                                                  | 2/2004           | Takiue            |                 |        |                       |
| FOREIGN PATENT DOCUMENTS                                                                                                                                         |                  |                   |                 |        |                       |
| EP                                                                                                                                                               | 1397304 A1       | 3/2004            |                 |        |                       |
| FR                                                                                                                                                               | 2197392          | 3/1974            |                 |        |                       |
| GB                                                                                                                                                               | 312464           | 5/1929            |                 |        |                       |
| JP                                                                                                                                                               | 169565           | 4/1971            |                 |        |                       |
| JP                                                                                                                                                               | S57161116 A      | 10/1982           |                 |        |                       |
| JP                                                                                                                                                               | 1260080          | 10/1989           |                 |        |                       |
| JP                                                                                                                                                               | 2242987          | 9/1990            |                 |        |                       |
| JP                                                                                                                                                               | 3033285          | 2/1991            |                 |        |                       |
| JP                                                                                                                                                               | 2000212884       | 8/2000            |                 |        |                       |
| JP                                                                                                                                                               | 2004126505       | 4/2004            |                 |        |                       |
| KR                                                                                                                                                               | 1019900010144    | 7/1990            |                 |        |                       |
| RU                                                                                                                                                               | 2100674          | 12/1997           |                 |        |                       |
| RU                                                                                                                                                               | 2295144          | 3/2007            |                 |        |                       |
| SU                                                                                                                                                               | 618061 A3        | 7/1978            |                 |        |                       |
| SU                                                                                                                                                               | 1647183          | 5/1991            |                 |        |                       |
| WO                                                                                                                                                               | 03102295         | 12/2003           |                 |        |                       |
| WO                                                                                                                                                               | 2004021771 A2    | 3/2004            |                 |        |                       |
| OTHER PUBLICATIONS                                                                                                                                               |                  |                   |                 |        |                       |
| Samson Rope Technologies, Inc., "Samson Deep Six Performs Beyond Expectation", Sep. 10, 2008, 2 pages.                                                           |                  |                   |                 |        |                       |
| Samson Rope Technologies, Inc., "Samson Offshore Expansion Celebrated", Feb. 18, 2009, 2 pages.                                                                  |                  |                   |                 |        |                       |
| USPTO, Office Action, U.S. Appl. No. 12/243,079, Jun. 28, 2010, 8 pages.                                                                                         |                  |                   |                 |        |                       |
| SLO, Response, U.S. Appl. No. 12/243,079, Oct. 28, 2010, 13 pages.                                                                                               |                  |                   |                 |        |                       |
| USPTO, Notice of Allowance, U.S. Appl. No. 12/243,079, Nov. 8, 2010, 16 pages.                                                                                   |                  |                   |                 |        |                       |
| SLO, Amendment After NOA, U.S. Appl. No. 12/243,079, Jan. 3, 2011, 4 pages.                                                                                      |                  |                   |                 |        |                       |
| USPTO, Issue Notification, U.S. Appl. No. 12/243,079, Mar. 2, 2011, 1 page.                                                                                      |                  |                   |                 |        |                       |
| USPTO, Office Action, U.S. Appl. No. 12/466,237, Mar. 10, 2011, 10 pages.                                                                                        |                  |                   |                 |        |                       |
| SLO, Response, U.S. Appl. No. 12/466,237, Jun. 10, 2011, 15 pages.                                                                                               |                  |                   |                 |        |                       |
| SLO, RCE, U.S. Appl. No. 12/466,237, Sep. 16, 2011, 1 page.                                                                                                      |                  |                   |                 |        |                       |
| US District Court, <i>Samson Rope Technologies, Inc. v. Yale Cordage, Inc.</i> Case 2:11-cv-00328, Document 1, Complaint (2), DI 001, Feb. 24, 2011, 5 pages.    |                  |                   |                 |        |                       |
| US District Court, <i>Samson Rope Technologies, Inc. v. Yale Cordage, Inc.</i> Case 2:11-cv-00328-JLR, Document 5, Notice to PTO, DI 005, Feb. 25, 2011, 1 page. |                  |                   |                 |        |                       |
| US District Court, <i>Samson Rope Technologies, Inc. v. Yale Cordage, Inc.</i> Case 2:11-cv-00328-JLR, Document 12, Answer, DI 012, May, 10, 2011, 6 pages.      |                  |                   |                 |        |                       |
| Herzog Braiding Machines, "Rope Braiding Machines Seng 140 Series", date unknown, 2 pages.                                                                       |                  |                   |                 |        |                       |
| Herzog Braiding Machines, "Rope Braiding Machines Seng 160 Series", date unknown, 2 pages.                                                                       |                  |                   |                 |        |                       |

**FIG. 1A****FIG. 1B**

FIG. 2



FIG. 3



FIG. 4



**FIG. 5****FIG. 6****FIG. 7****FIG. 8****FIG. 9****FIG. 10**

FIG. 11



FIG. 12



FIG. 13



FIG. 14



## WRAPPED YARNS FOR USE IN ROPES HAVING PREDETERMINED SURFACE CHARACTERISTICS

### RELATED APPLICATIONS

This application, U.S. patent application Ser. No. 14/262,600 filed Apr. 25, 2014 is a continuation of U.S. patent application Ser. No. 13/466,994 filed May 8, 2012, now U.S. Pat. No. 8,707,668 which issued on Apr. 29, 2014.

U.S. patent application Ser. No. 13/466,994 is a continuation of U.S. patent application Ser. No. 12/815,363 filed Jun. 14, 2010, now U.S. Pat. No. 8,171,713, which issued on May 8, 2012.

U.S. patent application Ser. No. 12/815,363 is a continuation of U.S. patent application Ser. No. 12/151,467 filed on May 6, 2008, now U.S. Pat. No. 7,735,308 which issued on Jun. 15, 2010.

U.S. patent application Ser. No. 12/151,467 is a continuation of U.S. patent application Ser. No. 11/599,817 filed on Nov. 14, 2006, now U.S. Pat. No. 7,367,176 which issued on May 6, 2008.

U.S. patent application Ser. No. 11/599,817 is a continuation of U.S. patent application Ser. No. 10/903,130 filed on Jul. 30, 2004, now U.S. Pat. No. 7,134,267 which issued on Nov. 14, 2006.

U.S. patent application Ser. No. 10/903,130 claims benefit of U.S. Provisional Application Ser. No. 60/530,132 filed on Dec. 16, 2003.

The contents of all related applications listed above are incorporated herein by reference.

### TECHNICAL FIELD

The present invention relates to rope systems and methods and, in particular, to wrapped yarns that are combined to form strands for making ropes having predetermined surface characteristics.

### BACKGROUND

The characteristics of a given type of rope determine whether that type of rope is suitable for a specific intended use. Rope characteristics include breaking strength, elongation, flexibility, weight, and surface characteristics such as abrasion resistance and coefficient of friction. The intended use of a rope will determine the acceptable range for each characteristic of the rope. The term “failure” as applied to rope will be used herein to refer to a rope being subjected to conditions beyond the acceptable range associated with at least one rope characteristic.

The present invention relates to ropes with improved surface characteristics, such as the ability to withstand abrasion or to provide a predetermined coefficient of friction. Typically, a length of rope is connected at first and second end locations to first and second structural members. Often, the rope is supported at one or more intermediate locations by intermediate structural surfaces between the first and second structural members. In the context of a ship, the intermediate surface may be formed by deck equipment such as a closed chock, roller chock, bollard or bit, staple, bullnose, or cleat.

When loads are applied to the rope, the rope is subjected to abrasion where connected to the first and second structural members and at any intermediate location in contact with an intermediate structural member. Abrasion and heat generated by the abrasion can create wear on the rope that can affect the performance of the rope and possibly lead to failure of the

rope. In other situations, a rope designed primarily for strength may have a coefficient of friction that is too high or low for a given use. The need thus exists for improved ropes having improved surface characteristics, such as abrasion resistance or coefficient of friction; the need also exists for systems and methods for producing such ropes.

### SUMMARY

10 The present invention may be embodied as a blended yarn comprising a plurality of first fibers and a plurality of second fibers. A coefficient of friction of the second fibers is greater than a coefficient of friction of the first fibers. Abrasion resistance characteristics of the second fibers are greater than abrasion resistance properties of the first fibers. A gripping ability of the second fibers is greater than a gripping ability of the first fibers. The plurality of second fibers are combined with the plurality of first fibers such that the first fibers extend along the length of the blended yarn and the second fibers do not extend along the length of the blended yarn and at least a portion of the second fibers are engaged with and extend from the plurality of first fibers effectively to define surface characteristics of the blended yarn.

25 The present invention may also be embodied as a rope adapted to engage a structural member, the rope comprising a plurality of wrapped yarns, where each wrapped yarn comprises a first set of first fibers and a second set of second fibers. The first set of the first fibers forms a core that is substantially surrounded by the second set. The first fibers are comprised of HMPE and substantially provide the load bearing characteristics of the rope. The second fibers are comprised of polyester and substantially provide abrasion resistance properties and gripping ability of the rope.

### BRIEF DESCRIPTION OF THE DRAWINGS

35 FIG. 1A is a side elevation view of a wrapped yarn that may be used to construct a rope of the present invention;

FIG. 1B is an end elevation cutaway view depicting the 40 yarn of FIG. 1A;

FIG. 2 is a side elevation view of a first example of a rope of the present invention;

FIG. 3 is a radial cross-section of the rope depicted in FIG. 2;

45 FIG. 4 is a close-up view of a portion of FIG. 3;

FIG. 5 is a side elevation view of a second example of a rope of the present invention;

FIG. 6 is a radial cross-section of the rope depicted in FIG. 5;

50 FIG. 7 is a close-up view of a portion of FIG. 6;

FIG. 8 is a side elevation view of a first example of a rope of the present invention;

FIG. 9 is a radial cross-section of the rope depicted in FIG. 8;

55 FIG. 10 is a close-up view of a portion of FIG. 9; and

FIG. 11 is a side elevation view of a first example of a rope of the present invention;

FIG. 12 is a radial cross-section of the rope depicted in FIG. 8;

60 FIG. 13 is a close-up view of a portion of FIG. 9; and

FIG. 14 is a schematic diagram representing an example process of fabricating the yarn depicted in FIGS. 1A and 1B.

### DETAILED DESCRIPTION

65 Referring initially to FIGS. 1A and 1B of the drawing, depicted therein is a blended yarn 20 constructed in accor-

dance with, and embodying, the principles of the present invention. The blended yarn **20** comprises at least a first set **22** of fibers **24** and a second set **26** of fibers **28**.

The first and second fibers **24** and **28** are formed of first and second materials having first and second sets of operating characteristics, respectively. The first material is selected primarily to provide desirable tension load bearing characteristics, while the second material is selected primarily to provide desirable abrasion resistance characteristics.

In addition to abrasion resistance, the first and second sets of operating characteristics can be designed to improve other characteristics of the resulting rope. As another example, certain materials, such as HMPE, are very slick (low coefficient of friction). In a yarn consisting primarily of HMPE as the first set **22** for strength, adding polyester as the second set **26** provides the resulting yarn **20** with enhanced gripping ability (increased coefficient of friction) without significantly adversely affecting the strength of the yarn **20**.

The first and second sets **22** and **26** of fibers **24** and **28** are physically combined such the first set **22** of fibers **24** is at least partly surrounded by the second set **26** of fibers **28**. The first fibers **24** thus form a central portion or core that is primarily responsible for bearing tension loads. The second fibers **28** form a wrapping that at least partly surrounds the first fibers **24** to provide the rope yarn **20** with improved abrasion resistance.

The example first fibers **24** are continuous fibers that form what may be referred to as a yarn core. The example second fibers **28** are discontinuous fibers that may be referred to as slivers. The term "continuous" indicates that individual fibers extend along substantially the entire length of the rope, while the term "discontinuous" indicates that individual fibers do not extend along the entire length of the rope.

As will be described below, the first and second fibers **24** and **28** may be combined to form the example yarn using a wrapping process. The example yarn **20** may, however, be produced using process for combining fibers into yarns other than the wrapping process described below.

With the foregoing understanding of the basic construction and characteristics of the blended yarn **20** of the present invention in mind, the details of construction and composition of the blended yarn **20** will now be described.

The first material used to form the first fibers **24** may be any one or more materials selected from the following group of materials: HMPE, LCP, or PBO fibers. The second material used to form the second fibers **28** may be any one or more materials selected from the following group of materials: polyester, nylon, Aramid, LCP, and HMPE fibers.

The first and second fibers **24** and **28** may be the same size or either of the fibers **24** and **28** may be larger than the other. The first fibers **24** are depicted with a round cross-section and the second fibers **28** are depicted with a flattened cross-section in FIG. 1B for clarity. However, the cross-sectional shapes of the fibers **24** and **28** can take forms other than those depicted in FIG. 1B. The first fibers **24** are preferably generally circular. The second fibers **28** are preferably also generally circular.

The following discussion will describe several particular example ropes constructed in accordance with the principles of the present invention as generally discussed above.

#### First Rope Example

Referring now to FIGS. 2, 3, and 4, those figures depict a first example of a rope **30** constructed in accordance with the principles of the present invention. As shown in FIG. 2, the rope **30** comprises a rope core **32** and a rope jacket **34**. FIG. 2

also shows that the rope core **32** and rope jacket **34** comprise a plurality of strands **36** and **38**, respectively. FIG. 4 shows that the strands **36** and **38** comprise a plurality of yarns **40** and **42** and that the yarns **40** and **42** in turn each comprise a plurality of fibers **44** and **46**, respectively.

One or both of the example yarns **40** and **42** may be formed by a yarn such as the abrasion resistant yarn **20** described above. However, because the rope jacket **34** will be exposed to abrasion more than the rope core **32**, at least the yarn **42** used to form the strands **38** should be fabricated at least partly from the abrasion resistant yarn **20** described above.

The exemplary rope core **32** and rope jacket **34** are formed from the strands **36** and **38** using a braiding process. The example rope **30** is thus the type of rope referred to in the industry as a double-braided rope.

The strands **36** and **38** may be substantially identical in size and composition. Similarly, the yarns **40** and **42** may also be substantially identical in size and composition. However, strands and yarns of different sizes and compositions may be combined to form the rope core **32** and rope jacket **34**.

As described above, fibers **44** and **46** forming at least one of the yarns **40** and **42** are of two different types. In the yarn **40** of the example rope **30**, the fibers **44** are of a first type corresponding to the first fibers **24** and a second type corresponding to the second fibers **28**. Similarly, in the yarn **42** of the example rope **30**, the fibers **46** are of a first type corresponding to the first fibers **24** and a second type corresponding to the second fibers **28**.

#### Second Rope Example

Referring now to FIGS. 5, 6, and 7, those figures depict a second example of a rope **50** constructed in accordance with the principles of the present invention. As perhaps best shown in FIG. 6, the rope **50** comprises a plurality of strands **52**. FIG. 7 further illustrates that each of the strands **52** comprises a plurality of yarns **54** and that the yarns **54** in turn comprise a plurality of fibers **56**.

The example yarn **54** may be formed by a yarn such as the abrasion resistant yarn **20** described above. In the yarn **54** of the example rope **50**, the fibers **56** are of a first type corresponding to the first fibers **24** and a second type corresponding to the second fibers **28**.

The strands **52** are formed by combining the yarns **54** using any one of a number of processes. The exemplary rope **50** is formed from the strands **52** using a braiding process. The example rope **50** is thus the type of rope referred to in the industry as a braided rope.

The strands **52** and yarns **54** forming the rope **50** may be substantially identical in size and composition. However, strands and yarns of different sizes and compositions may be combined to form the rope **50**. The first and second types of fibers combined to form the yarns **54** are different as described above with reference to the fibers **24** and **28**.

#### Third Rope Example

Referring now to FIGS. 8, 9, and 10, those figures depict a third example of a rope **60** constructed in accordance with the principles of the present invention. As perhaps best shown in FIG. 9, the rope **60** comprises a plurality of strands **62**. FIG. 10 further illustrates that each of the strands **62** in turn comprises a plurality of yarns **64**, respectively. The yarns **64** are in turn comprised of a plurality of fibers **66**.

The example yarn **64** may be formed by a yarn such as the abrasion resistant yarn **20** described above. The fibers **66** of at least some of the yarns **64** are of a first type and a second type,

where the first and second types and correspond to the first and second fibers 24 and 28, respectively.

The strands 62 are formed by combining the yarns 64 using any one of a number of processes. The exemplary rope 60 is formed from the strands 62 using a twisting process. The example rope 60 is thus the type of rope referred to in the industry as a twisted rope.

The strands 62 and yarns 64 forming the rope 60 may be substantially identical in size and composition. However, strands and yarns of different sizes and compositions may be combined to form the rope 60. The first and second types of fibers are combined to form at least some of the yarns 64 are different as described above with reference to the fibers 24 and 28.

#### Fourth Rope Example

Referring now to FIGS. 11, 12, and 13, those figures depict a fourth example of a rope 70 constructed in accordance with the principles of the present invention. As perhaps best shown in FIG. 12, the rope 70 comprises a plurality of strands 72. FIG. 13 further illustrates that each of the strands 72 comprise a plurality of yarns 74 and that the yarns 74 in turn comprise a plurality of fibers 76, respectively.

One or both of the example yarns 74 may be formed by a yarn such as the abrasion resistant yarn 20 described above. In particular, in the example yarns 74 of the example rope 70, the fibers 76 are each of a first type corresponding to the first fibers 24 and a second type corresponding to the second fibers 28.

The strands 72 are formed by combining the yarns 74 using any one of a number of processes. The exemplary rope 70 is formed from the strands 72 using a braiding process. The example rope 70 is thus the type of rope commonly referred to in the industry as a braided rope.

The strands 72 and yarns 74 forming the rope 70 may be substantially identical in size and composition. However, strands and yarns of different sizes and compositions may be combined to form the rope 70. The first and second types of fibers are combined to form at least some of the yarns 74 are different as described above with reference to the fibers 24 and 28.

#### Yarn Fabrication

Turning now to FIG. 14 of the drawing, depicted at 120 therein is an example system 120 for combining the first and second fibers 24 and 28 to form the example yarn 20. The system 120 basically comprises a transfer duct 122, a convergence duct 124, a suction duct 126, and a false-twisting device 128. The first fiber 24 is passed between a pair of feed rolls 130 and into the convergence duct 124. The second fiber 28 is initially passed through a pair of back rolls 142, a pair of drafting aprons 144, a pair of drafting rolls 146, and into the transfer duct 122.

The example first fibers 24 are continuous fibers that extend substantially the entire length of the example yarn 20 formed by the system 120. The example second fibers 28 are slivers, or discontinuous fibers that do not extend the entire length of the example yarn 20.

The second fibers 28 become airborne and are drawn into convergence duct 124 by the low pressure region within the suction duct 126. The first fibers 24 converge with each other and the airborne second fibers 28 within the convergence duct 124. The first fibers 24 thus pick up the second fibers 28. The first and second fibers 24 and 28 are then subsequently twisted by the false-twisting device 128 to form the yarn 20. The twist

is removed from the first fibers 24 of the yarn 20 as the yarn travels away from the false-twisting device 128.

After the yarn 20 exits the false-twisting device 128 and the twist is removed, the yarn passes through let down rolls 150 and is taken up by a windup spool 152. A windup roll 154 maintains tension of the yarn 20 on the windup spool 152.

#### First Yarn Example

10 A first example of the yarn 20 that may be fabricated using the system 120 as described above comprises the following materials. The first fibers 24 are formed of HMPE fibers and the second fibers are formed of polyester fibers. The yarn of the first example comprises between about sixty to eighty percent by weight of the first fibers 24 and between about twenty to forty percent by weight of the second fibers 28.

#### Second Yarn Example

20 A second example of the yarn 20 that may be fabricated using the system 120 as described above comprises the following materials. The first fibers 24 are formed of LCP fibers and the second fibers are formed of a combination of LCP fibers and Aramid fibers. The yarn of the second example comprises between about fifteen and thirty-five percent by weight of the first fibers 24 and between about sixty-five and eighty-five percent by weight of the second fibers 28. More specifically, the second fibers 28 comprise between about forty and sixty percent by weight of LCP and between about forty and sixty percent by weight of Aramid.

Given the foregoing, it should be clear to one of ordinary skill in the art that the present invention may be embodied in other forms that fall within the scope of the present invention.

What is claimed is:

- 35 1. A method of forming a blended yarn adapted to engage first and second structural members comprising the steps of: providing a plurality of first fibers, where the first fibers are sized to extend along a length of the blended yarn; and providing a plurality of second fibers, where the second fibers are sized to extend only partly along a length of the blended yarn, a coefficient of friction of the second fibers is greater than a coefficient of friction of the first fibers, abrasion resistance characteristics of the second fibers are greater than abrasion resistance properties of the first fibers, and a gripping ability of the second fibers is greater than a gripping ability of the first fibers; forming a combination of the plurality of first fibers and the plurality of second fibers by passing the plurality of first fibers and the plurality of second fibers through a convergence duct such that the first fibers pick up the second fibers; imparting a false twist to the combination of the plurality of first fibers and the plurality of second fibers by passing the combination of the plurality of first fibers and the plurality of second fibers through a false-twisting device; removing the false twist from the combination of the plurality of first fibers and the plurality of second fibers to form the blended yarn; and arranging at least portion of the blended yarn against the first and second structural members such that tension loads are applied on the blended yarn by the first and second structural members, where the tension loads on the blended yarn are primarily borne by the first fibers, and

where the blended yarn engages the first and second structural members, the second fibers substantially determine friction, abrasion resistance, and gripping ability of the blended yarn.

2. A method as recited in claim 1, in which at least a portion of the second fibers are engaged with and extend from the plurality of first fibers to define surface characteristics of the blended yarn.

3. A method as recited in claim 1, in which step of forming the combination of the plurality of first fibers and the plurality of second fibers comprises the step of arranging the second fibers to at least partly surround the first fibers.

4. A method as recited in claim 1, in which step of forming the combination of the plurality of first fibers and the plurality of second fibers comprises the step of forming a core comprising the first fibers, where the second fibers surround the first fibers.

5. A method as recited in claim 1, in which the second fibers comprise at least one fiber selected from the group of fibers consisting of polyester, nylon, Aramid, LCP, and HMPE fibers.

6. A method as recited in claim 1, in which the second fibers are polyester fibers.

7. A method as recited in claim 6, in which the blended yarn comprises about sixty to eighty percent by weight of the first fibers and about twenty to forty percent by weight of the second fibers.

8. A method as recited in claim 1, in which the second fibers are LCP and Aramid fibers.

9. A method as recited in claim 8, in which the blended yarn comprises about fifteen to thirty-five percent by weight of the first fibers and about sixty-five to eighty five percent by weight of the second fibers.

10. A method as recited in claim 1, in which the first fibers are HMPE fibers.

11. A method as recited in claim 1, further comprising the step of forming a braided rope formed from a plurality of blended yarns.

12. A method as recited in claim 11, in which the step of forming the braided rope further comprises the step of forming a core and a jacket.

13. A method as recited in claim 11, in which the step of forming the braided rope further comprises the step of forming a double braided rope.

14. A method as recited in claim 1, further comprising the steps of:

combining a plurality of the blended yarns to form a plurality of strands; and

combining the plurality of strands are combined to form a rope.

15. A method of forming a rope adapted to engage first and second structural members, the method comprising the steps of:

providing a first set of first fibers;

providing a second set of second fibers;

combining the first and second sets of fibers to form a plurality of wrapped yarns such that the first set of the first fibers forms a core that is substantially surrounded by the second set,

the first fibers substantially determine the load bearing characteristics of the rope, and

the second fibers substantially determine abrasion resistance properties and gripping ability of the rope; and arranging at least a portion of the rope against the first and second structural members such that

tension loads are applied on the rope by the first and second structural members, where the tension loads on the rope are primarily borne by the first fibers, and where the rope engages the first and second structural members, the second fibers substantially determine friction, abrasion resistance, and gripping ability of the rope.

16. A method as recited in claim 15, in which the first fibers are formed of HMPE and the second fibers are formed of polyester.

17. A method of forming a blended yarn adapted to engage first and second structural members comprising the steps of:

selecting a plurality of first fibers and a plurality of second fibers such that

a coefficient of friction of the second fibers is greater than a coefficient of friction of the first fibers, abrasion resistance characteristics of the second fibers are greater than abrasion resistance properties of the first fibers, and

a gripping ability of the second fibers is greater than a gripping ability of the first fibers;

combining the plurality of second fibers with the plurality of first fibers using a false-twisting process such that the first fibers extend along the length of the blended

yarn and the second fibers do not extend along the length of the blended yarn, and

at least a portion of the second fibers are engaged with and extend from the plurality of first fibers effectively to define surface characteristics of the blended yarn; and

arranging at least a portion of the blended yarn against the first and second structural members such that

tension loads are applied on the blended yarn by the first and second structural members, where the tension loads on the blended yarn are primarily borne by the first fibers, and

where the blended yarn engages the first and second structural members, the second fibers substantially determine friction, abrasion resistance, and gripping ability of the blended yarn.

18. A method as recited in claim 17, in which the second fibers at least partly surround the first fibers.

19. A method as recited in claim 17, in which at least a plurality of the first fibers are continuous and at least a plurality of the second fibers are discontinuous.